

# UNITED STATES PATENT OFFICE.

MARY AUGUSTA HUNTER, OF PHILADELPHIA, PENNSYLVANIA.

## PROCESS OF CONVERTING IRON CASTINGS INTO STEEL OR MALLEABLE IRON.

No. 846,081.

Specification of Letters Patent.

Patented March 5, 1907.

Application filed March 28, 1906. Serial No. 308,576.

*To all whom it may concern:*

Be it known that I, MARY AUGUSTA HUNTER, of the city of Philadelphia, in the county of Philadelphia and State of Pennsylvania, have invented certain new and useful Improvements in Processes of Converting Iron Castings into Steel or Malleable Iron, of which the following is a specification.

My invention relates to improvements in processes for converting iron castings into steel or malleable iron; and the objects of my invention are to convert cast-iron as quickly and as cheaply as possible without remelting into a steel capable of being rolled, hammered, or drawn like wrought-iron or low-carbon steel and which can be tempered the same as high-grade tool-steel, further objects being to eliminate the suffocating fumes which have hitherto been prevalent in former processes of this nature and to obtain a resulting product which shall possess little, if any, scale on the surface thereof; and it consists, essentially, of subjecting the iron when heated to a point slightly short of melting to the action of sulfuric acid in gaseous or liquid form, the various steps of the process being hereinafter described in detail.

In carrying out the process I first place the cast-iron, which may be in the form of castings, bars, or blocks, into a suitable muffle-furnace or other receptacle, in which it may be heated to a high temperature.

While not limiting my process to any particular type of furnace, I find it can be used with particular advantage in the furnace which is covered by the United States Patent No. 699,759, granted to J. A. Hunter on the 13th day of May, 1902. In this furnace a special provision is made for carrying out a process analogous to this one. The iron in the furnace is then heated to a high temperature short of melting-point. I usually find that a temperature between 1,700° and 1,800° Fahrenheit is suitable for the carrying out of my process. After the iron has been heated to this high temperature it is treated with sulfuric acid in the form of a vapor or spray. It will be evident that this sulfuric acid may be applied to the iron in many different ways, the essential point being that the acid come in contact with the iron at the high temperature. I may, however, mention one or two ways in which they may be carried out.

First, it might be carried out by the means shown and described in United States Patent No. 699,759, in which the acid is introduced in puffs through openings in the muffle to the iron when the proper temperature has been obtained. The high temperature of the furnace vaporizes the acid, and the fumes thereof rise up and come in contact with the iron castings or ingots.

Secondly, the acid might be introduced in the form of a spray by compressed air. Apparatus for carrying out this method is quite well known to those familiar with the art and need not be here described.

Thirdly, the sulfuric acid might previously be vaporized externally to the furnace and forced into the furnace by its own pressure.

The theoretical operation of my process as I at present conceive it is as follows: The sulfuric-acid vapor coming in contact with the iron at a high temperature decomposes, giving off oxygen. The oxygen burning the impurities in the iron raises the temperature of the furnace still higher, causing a molecular change to take place in the structure of the iron, as well as the chemical change due to the burning of the impurities. The physical change which takes place in the iron comprises a recrystallization in the structure of the iron and a conversion of a portion of the carbon into carbon of a different form—namely, into the carbon of cementation—and an elimination of part of the combined carbon. In this physical transformation the molecules of the iron thus become more or less granulated, and the carbon of cementation acts as a binder to join the granules more closely together. The tensile strength and ductility of the metal is thus greatly increased.

By variation in the proportion of the acid introduced into the furnace the nature of the finished product may be varied, according as steel, malleable iron, or wrought-iron is desired.

The metal which is produced by my process as hereinbefore described possesses the peculiar properties of being capable of being rolled, hammered, and drawn equally well as ordinary wrought-iron or low-carbon steel and at the same time can be tempered equally well as high-grade tool-steel.

The method of heating the iron or the method of introducing the acid to the iron do not form essential features of my process, and it is manifest that these can be carried 5 out in a great variety of different ways, the main feature being the application of the acid to the iron at a high temperature.

What I claim as my invention is—

10 The mode herein described of converting cast-iron into steel or malleable iron consisting in heating the iron in a closed chamber, to a point slightly short of the melting-point

of the iron; then introducing into the chamber sulfuric acid unmixed with any other reducing agent and continuing the heating, effecting the decomposition of the sulfuric acid and enabling the oxygen therein to act on the iron substantially as described. 15

Signed at Philadelphia, Pennsylvania, this 23d day of March, 1906.

MARY AUGUSTA HUNTER.

Witnesses:

THOS. H. MAGINNIS,  
A. B. PECK.